

1

2,932,942

## JET FUEL COMPOSITIONS

George G. Ecke, Ferndale, Mich., and Alfred J. Kolka, Clairton, Pa., assignors to Ethyl Corporation, New York, N.Y., a corporation of Delaware

No Drawing. Application January 22, 1957  
Serial No. 635,147

7 Claims. (Cl. 60—35.4)

This invention relates to new jet fuel compositions characterized by high thermal stability.

Fuel temperatures in modern jet aircraft power plants are becoming so high that harmful deposits are formed in the precombustion phase of the fuel system. Contributing to this has been the use of the fuel as a heat sink to aid in lubricating oil cooling, which has increased fuel temperatures to the point where deposits are so severe that they interfere with normal fuel combustion as well as lubricating oil temperature control. The jet fuel thermal stability problem is so serious that it can eventually lead to engine failure of the turbine section due to uneven temperature patterns. In fact, it is considered the outstanding problem in jet fuels at the present time.

Prior investigators have found that conventional gasoline antioxidants are incapable of overcoming this oppressive problem. The art is replete with reports by eminent investigators which are universally to the effect that conventional antioxidants do not overcome the jet fuel thermal stability problem. For example, it has been stated that neither 4-methyl-2,6-di-*tert*-butyl phenol nor N,N'-di-*sec*-butyl-p-phenylenediamine improves the high-temperature stability of jet fuels. In fact, some gasoline antioxidants have been shown to be deleterious in that they increase the severity of the problem. Consequently, the experts in the field have turned their attention to other types of additives—i.e., materials which are not antioxidants. One approach has been the use of dispersants in an attempt to keep the deposits suspended in the fuel and thereby prevent them from adhering to critical engine surfaces. However, this approach has not proved satisfactory because the deterioration of the fuel does occur under jet engine operating conditions and little, if any, improvement in engine performance has as yet been attained. Another approach has been the use of various jet fuel treating procedures. However, these are unsatisfactory because they are expensive and complicated and, in most cases, little improvement is achieved. Special fuel blending procedures have also been suggested but found totally impractical. Thus, in general, all approaches to the solution of this substantial problem have thus far been unsuccessful.

An object of this invention is to alleviate the thermal stability problems in jet fuels. Another object is to provide new jet fuel compositions which are characterized by a high degree of thermal stability. A further object is to overcome the thermal instability problems in jet fuels in a simple and inexpensive manner. A still further object is to provide processes of inhibiting deterioration of jet fuel normally tending to occur at elevated temperatures below the cracking temperatures of the fuel. Other objects will be apparent from the ensuing description.

It has been found that the above and other objects of this invention are accomplished by providing jet fuel containing from about 0.001 to about 0.5 percent by weight—preferably from about 0.01 to about 0.1 per-

2

cent—of a 4-amino-2,6-dihydrocarbon-substituted phenol having the general formula:



wherein R<sub>1</sub> and R<sub>2</sub> are alkyl, cycloalkyl, or aralkyl groups containing up to about 12 carbon atoms each and R<sub>3</sub> and R<sub>4</sub> are alkyl, cycloalkyl, or aralkyl groups containing up to about 8 carbon atoms, or hydrogen. The thermal stabilizers of this invention have the surprising faculty of greatly improving the thermal stability of jet fuels and this effectiveness is independent of the hydrocarbon types from which the jet fuel has been prepared. Thus, the present invention affords extreme protection against thermal instability of all present-day jet fuels.

While all of the compounds defined by the above general formula give very good results, a preferred class comprises those compounds in which R<sub>1</sub> is an alkyl group containing no more than about 12 carbon atoms, R<sub>2</sub> is a tertiary alkyl group containing 4 to 5 carbon atoms, and R<sub>3</sub> and R<sub>4</sub> are alkyl, cycloalkyl, or aralkyl groups containing no more than about 8 carbon atoms, or hydrogen. These preferred compounds are characterized by being insoluble in water and in dilute aqueous alkali solutions, and highly soluble in jet fuel. Thus, these compounds remain dissolved in the fuel even though it is treated with aqueous caustic washes or is stored over or comes in contact with water. Thus, the preferred jet fuels of this invention are not deprived of their thermal stabilizer content during commercially used refinery steps, such as caustic treatments, aqueous washes, or storage and transportation operations involving contact with water. These preferred compounds are also characterized by being exceptionally effective jet fuel thermal stabilizers.

Particularly preferred jet fuel additives of this invention are those in which R<sub>1</sub> is an alkyl group containing no more than about 12 carbon atoms, R<sub>2</sub> is a tertiary butyl group, and R<sub>3</sub> and R<sub>4</sub> are hydrogen. These particularly preferred compounds are easily prepared at low cost from readily available, inexpensive starting materials and are the most outstandingly effective jet fuel thermal stabilizers.

Referring to the above general formula, it is seen that the jet fuel additives of this invention are characterized by having hydrocarbon substituents in both positions ortho to the hydroxyl group and by having an unsubstituted amino, mono-substituted amino, or di-substituted amino group in the para position. The particular structural requirements of these compounds impart to them a community of properties of extreme value in the thermal stabilization of jet fuels.

The jet fuel additives of this invention directly attack and overcome the thermal instability problem at its source. They confer very high thermal stability upon the finished fuels of this invention so that the fuels strongly resist thermally-induced degradation. Thus, markedly reduced is the amount of insoluble thermal decomposition products which heretofore deposited to plug orifices in the fuel system, to distort fuel flow and thus impair flame pattern, and to foul surfaces. Furthermore, the additives of this invention do not introduce secondary problems in use, such as jet fuel foaming at high altitudes, emulsification difficulties, interference with low-temperature flows, and the like. At the same time, all of these highly-

important and unique advantages are achieved in a simple manner and at very low cost.

It is known that conventional jet fuel normally tends to deteriorate when subjected to the condition of elevated temperatures below the cracking temperature of the fuel, i.e., temperatures in the range of about 300 to 500° F. Hence, another part of this invention is the process of inhibiting such deterioration which comprises subjecting to this condition a jet fuel containing from about 0.001 to about 0.5 (and preferably from about 0.01 to about 0.1) percent by weight of a 4-amino-2,6-dihydrocarbon-substituted phenol as defined by the above general formula. Thus, greatly enhanced thermal stability of jet fuel is achieved by blending with a jet fuel these concentrations of a 4-amino-2,6-dihydrocarbon-substituted phenol additive of this invention, especially one of the preferred types, and subjecting the resulting fuel to the above condition.

The jet fuels whose thermal stability is greatly improved pursuant to this invention are principally hydrocarbon fuels which are heavier than gasoline, i.e., distilled liquid hydrocarbon fuels having a higher endpoint than gasoline. In general, the jet fuels can be comprised of distillate fuels and naphthas and blends of the above, including blends with lighter hydrocarbon fractions, so long as the endpoint of the final jet fuel is at least 435° F. and preferably greater than 480° F. It will be understood, however, that the jet fuels which are employed according to this invention can contain certain other ingredients, such as alcohols or the like, provided the resulting fuel blend meets the specifications imposed upon jet fuels.

Typical jet fuels improved according to this invention include JP-3, a mixture of about 70 percent gasoline and 30 percent light distillate having a 90 percent evaporated point of 470° F.; JP-4, a mixture of about 65 percent gasoline and 35 percent light distillate—a fuel especially designed for high altitude performance; JP-5, an especially fractionated kerosene; high flash point-low freezing point kerosene, etc.

The following are specifications of typical liquid hydrocarbon jet fuels of this invention:

|                                     | Fuel A<br>(JP-3) | Fuel B<br>(JP-4) | Fuel C<br>(JP-5) | Fuel D<br>(JP-4) | Fuel E<br>(JP-4<br>referee) | Fuel F<br>(Kero-<br>sene) |
|-------------------------------------|------------------|------------------|------------------|------------------|-----------------------------|---------------------------|
| 10% Evaporated,<br>°F.              | 160              | 220              | 395              | 221              | —                           | 380                       |
| 90% Evaporated,<br>°F.              | 470              | 470              | 480              | 379              | 460                         | 480                       |
| Endpoint, °F.                       | 600              | 550              | 550              | 480              | 516                         | 48                        |
| Gravity, API                        | 50               | 45               | 35               | 47.3             | 48.5                        | 43                        |
| Existent Gum,<br>mg./100 ml., max.  | 7                | 7                | 7                | 1.0              | 1.4                         | 1.7                       |
| Potential Gum,<br>mg./100 ml., max. | 14               | 14               | 14               | 1.0              | 9.6                         | —                         |
| Reid Vapor Pres-<br>sure, p.s.i.    | 7.0              | 3.0              | —                | —                | —                           | —                         |
| Aromatics, vol.<br>percent          | 25.0             | 25.0             | 25.0             | 12.5             | 14.6                        | 14.3                      |
| Olefins, vol. percent               | 5.0              | 5.0              | 5.0              | 0.3              | 1.2                         | —                         |

The following examples illustrate various specific embodiments of this invention.

#### EXAMPLE 1

To 100,000 parts of fuel A is added with stirring 10 parts (0.01 percent) of 4-amino-2,6-dimethyl phenol dissolved in 200 parts of ethanol. The resulting fuel is found to possess improved thermal stability characteristics.

#### EXAMPLE 2

To 100,000 parts of fuel B is added 100 parts (0.1 percent) of 4-(N,N-diethylamino)-2,6-di-(2-dodecyl) phenol dissolved in 500 parts of methanol. The resulting fuel possesses improved thermal stability properties.

#### EXAMPLE 3

With 100,000 parts of fuel C is blended 50 parts (0.05 percent) of 4-(N-isobutylamino)-2,6-dicyclohexyl phenol.

The resulting fuel blend possesses superior thermal stability characteristics.

#### EXAMPLE 4

To 100,000 parts of fuel D is added 40 parts (0.04 percent) of 4-amino-2,6-di-(1-phenylethyl) phenol dissolved in 400 parts of toluene. The resulting fuel blend is found to possess superior thermal stability characteristics.

#### EXAMPLE 5

With 100,000 parts of fuel E is blended 80 parts (0.08 percent) of 4-(N-cyclohexylamino)-2,6-diisopropyl phenol. The resulting fuel blend possesses enhanced thermal stability properties.

#### EXAMPLE 6

To 100,000 parts of fuel F is added 2 parts (0.002 percent) of 4-(N,N-dibenzylamino)-2,6-diethyl phenol dissolved in 50 parts of isopropanol. The resulting fuel blend is found to possess enhanced thermal stability properties.

#### EXAMPLE 7

Fuel C is blended with a lighter hydrocarbon fraction to give a final jet fuel having an endpoint of 435° F. To 100,000 parts of the resultant fuel is added with stirring 500 parts (0.5 percent) of 4-(N-methyl-N-isopropylamino)-2-methyl-6-isopropyl phenol. The resulting fuel possesses improved thermal stability characteristics.

#### EXAMPLE 8

To 100,000 parts of a liquid hydrocarbon jet fuel having an endpoint of 550° F. is added 300 parts (0.3 percent) of 4-(N,N-dibutylamino)-2-methyl-6-cyclohexyl phenol dissolved in 2500 parts of mixed xylenes. The resulting jet fuel possesses superior thermal stability properties.

#### EXAMPLE 9

With 100,000 parts of fuel A is blended 6 parts (0.006 percent) of 4-(N-(4-methylbenzyl)-N-ethylamino)-2,6-di-(2-hexyl) phenol. This fuel, after mixing, possesses improved thermal stability characteristics.

#### EXAMPLE 10

70 parts of 4-amino-2,6-di-(3-decyl)-phenol is blended with 100,000 parts of fuel B. The resulting jet fuel containing 0.07 percent of the phenol possesses improved thermal stability characteristics.

#### EXAMPLE 11

With 100,000 parts of fuel C is blended 50 parts (0.05 percent) of 4-(N-ethylamino)-2-methyl-6-tert-butyl phenol. The resulting jet fuel blend possesses greatly superior thermal stability characteristics.

#### EXAMPLE 12

To 100,000 parts of fuel D is added with stirring 20 parts (0.02 percent) of 4-(N-cyclohexylamino)-2-ethyl-6-tert-amyl phenol. The resulting jet fuel is found to possess vastly superior thermal stability characteristics.

#### EXAMPLE 13

With 100,000 parts of fuel E is blended 200 parts (0.2 percent) of 4-(N-benzylamino)-2,6-di-tert-butyl phenol. The resulting jet fuel blend possesses markedly superior thermal stability properties.

#### EXAMPLE 14

To 100,000 parts of fuel F is added with stirring 50 parts (0.05 percent) of 4-(N,N-dimethylamino)-2-isopropyl-6-tert-butyl phenol. The resulting fuel possesses vastly superior thermal stability characteristics.

#### EXAMPLE 15

With 100,000 parts of fuel A is blended 100 parts (0.1 percent) of 4-(N-cyclohexyl)-N-ethylamino-2-(2-dodecyl)

yl)-6-tert-amyl phenol. The resultant jet fuel is found to possess greatly superior thermal stability characteristics.

EXAMPLE 16

With 100,000 parts of fuel B is blended 80 parts (0.08 percent) of 4-amino-2,6-di-tert-butyl phenol. The resulting jet fuel possesses outstanding thermal stability characteristics.

EXAMPLE 17

To 100,000 parts of fuel C is added with stirring 50 parts (0.05 percent) of 4-amino-2-methyl-6-tert-butyl phenol. The resulting jet fuel possesses elegant thermal stability properties.

EXAMPLE 18

With 100,000 parts of fuel D is blended 100 parts (0.1 percent) of 4-amino-2-isopropyl-6-tert-butyl phenol. The resulting jet fuel possesses outstandingly superior thermal stability characteristics.

EXAMPLE 19

To 100,000 parts of fuel E is added with stirring 60 parts (0.06 percent) of 4-amino-2-(2-hexyl)-6-tert-butyl phenol. Outstanding thermal stability properties are possessed by the resulting fuel.

EXAMPLE 20

To 100,000 parts of fuel F is added with stirring 50 parts (0.05 percent) of 4-amino-2-(2-dodecyl)-6-tert-butyl phenol. Outstandingly superior thermal stability properties are possessed by the resulting fuel.

Examples 11 through 15 illustrate preferred jet fuels of this invention containing preferred 4-amino-2,6-dialkyl phenols. Particularly preferred jet fuels of this invention are illustrated by Examples 16 through 20, since the fuels in these examples contain particularly preferred 4-amino-2,6-dialkyl phenols.

The improvements resulting from the use of the additives of this invention in jet fuels are demonstrated by tests in an apparatus known as the Coordinating Fuel Research (CFR) Jet Fuel Coker, commonly called the "Erdco Rig." See Petroleum Processing, December, 1955, pages 1909-1911. For these tests the apparatus was modified to permit concurrent determination of both the filter plugging characteristics and the preheater deposit-forming tendencies of the test fuels. This was done by providing a by-pass line around the filter, valved so that the fuel was passed through the filter until either the test was completed with a pressure drop across the filter of less than 25 inches of mercury, or until this pressure drop occurred during the test period. In the latter instance, the valve was immediately adjusted so that the fuel by-passed the filter thereby enabling the continuation of the test for the predetermined period so as to measure the amount of preheater tube deposits formed during the entire test period. The test conditions consisted of maintaining the preheater temperature at 400° F., the filter temperature at 500° F., and the fuel flow rate at six pounds per hour. Since the temperature of the preheater is essentially independent of the filter temperature, the filter heater was turned off whenever the by-pass was used. Each test was carried out for a period of 150 minutes.

The jet fuel base stock used in these tests was a commercially-available JP-5 fuel of very poor thermal stability. The inspection data on this fuel are shown in the following table:

|                                  |      |
|----------------------------------|------|
| Gravity, °API                    | 39.0 |
| Distillation, ASTM D86:          |      |
| Temp., °F. at percent recovered— |      |
| Start                            | 360  |
| 5                                | 377  |
| 10                               | 381  |
| 20                               | 392  |
| 30                               | 400  |

6  
Distillation, ASTM D86—Continued

|    | Temp., °F. at percent recovered—      | Continued |
|----|---------------------------------------|-----------|
| 5  | 40                                    | 410       |
|    | 50                                    | 419       |
|    | 60                                    | 430       |
|    | 70                                    | 443       |
|    | 80                                    | 458       |
|    | 90                                    | 480       |
|    | 95                                    | 499       |
|    | Endpoint                              | 524       |
|    | Recovered, percent                    | 98        |
|    | Residue, percent                      | 1         |
|    | Loss, percent                         | 1         |
|    | Flash, PM, °F.                        | 148       |
| 15 | Aniline point                         | 132       |
|    | Aniline-gravity constant              | 5148      |
|    | Hydrocarbon type analysis, FIAM:      |           |
|    | Aromatic, vol. percent                | 16        |
|    | Olefins, vol. percent                 | 0         |
| 20 | Saturates, vol. percent               | 84        |
|    | Viscosity, cs. at -30° F.             | 10.65     |
|    | Freezing point, °F.                   | -42       |
|    | Existent gum, mg./100 ml. (steam jet) | -42       |
|    | Potential gum, mg./100 ml.            | 1         |
| 25 | Total sulfur, wt. percent             | 0.052     |
|    | Mercaptan sulfur, wt. percent         | <0.001    |
|    | Smoke point, mm.                      | 19        |
|    | Water reaction                        | 1B        |
| 30 | Water tolerance                       | OK, 1 ml. |

With one portion of this base fuel was blended 4-amino-2,6-di-tert-butyl phenol at a concentration of 0.027 percent by weight. Another portion of this base fuel was treated with an identical concentration of 4-amino-2-methyl-6-tert-butyl phenol. These fuels as well as the additive-free base fuel were then subjected to the above test. Measured were the pressure drop across the filter—which is directly related to the filter plugging characteristics of the fuel, hence, its thermal stability—and the preheater deposit-forming tendencies of the test fuels. The nature of the deposits formed on the preheater tube surfaces is also a direct measure of the thermal stability of the fuel. Accordingly, if a light-colored deposit is formed, only a small amount of high temperature deterioration of the fuel has occurred. Thus, the darker the deposits, the more thermally unstable is the fuel. An additional criterion of the thermal stability of the fuel is the merit rating the fuel possessed on completion of the test. In the merit rating system a value of 900 represents perfect fuel performance—i.e., no pressure drop in 300 minutes—whereas a zero rating is achieved when the fuel exhibits a pressure drop of 25 inches of mercury in zero time. Thus, the nearer the merit rating to 900, the more nearly perfect is the fuel. The results of these tests are shown in the following table, the 4-amino-2,6-di-tert-butyl phenol and 4-amino-2-methyl-6-tert-butyl phenol being designated therein additives A and B, respectively.

Table.—Effect of additives on the thermal stability of jet fuel

| Additive | Filter Test Time, min. | Pressure Drop Across Filter, In. of Hg | Merit Rating | Preheater Deposit Characteristics                                                                          |
|----------|------------------------|----------------------------------------|--------------|------------------------------------------------------------------------------------------------------------|
| None     | 25                     | 25                                     | 48           | Preheater tube coated with heavy, dark-brown and black deposits.                                           |
| A        | 150                    | 0.1                                    | ca. 800      | Preheater tube coated with a barely perceptible haze and a very small amount of very light-brown deposits. |
| B        | 150                    | 0.1                                    | ca. 800      | Preheater tube coated with a barely perceptible light haze and a trace of very light tan deposits.         |

The data in the above table are illustrative of the improved thermal stability characteristics of jet fuels caused by the presence therein of the preferred additives of this invention. Thus, on the basis of filter plugging time, improvements which defy quantitative expression were achieved by the practice of this invention. This is shown by the fact that a pressure drop of 25 inches of mercury occurred within the first 25 minutes of the test time when using the additive-free base fuel; whereas both of the fuels of this invention ran through the entire test period and only exhibited a pressure drop of 0.1 inch of mercury. Furthermore, the merit ratings which, as pointed out above, are correlated to the thermal stability of the fuels in terms of filter plugging and time show the enormous benefits achieved by blending with jet fuel the particularly preferred additives of this invention. Thus, while the base fuel had a very low merit rating of 48, both of the above illustrative particularly preferred fuels of this invention had merit ratings of 800 (extrapolated to 300 minutes) which places them in the category of nearly perfect fuel performance. From the standpoint of preheater deposits, the fuels of this invention likewise exhibited tremendously improved properties because not only were the heavy, dark-brown to black deposits of the base fuel completely eliminated, but the deposits formed from the fuels of this invention were almost entirely in the form of a barely perceptible haze. So far as we are aware, never before have additives given such exceptional effectiveness insofar as the jet fuel thermal instability problem is concerned.

To illustrate the very great improvements in jet fuel thermal stability brought about by other additives of this invention which are not even of the preferred type, the above test was conducted on the base fuel containing 0.014 percent by weight of 4-(N-sec-butylamino)-2,6-di-isopropyl phenol. At this very low concentration, this additive almost doubled the filter test time and the merit rating as compared with the additive-free base fuel. Moreover, only a very small amount of preheater tube deposits were formed, most of which were in the form of a barely perceptible haze with only a trace quantity of a brown deposit being detectable. Thus, these results show not only that very good results are achieved by using the non-preferred additives of this invention, but serve to point up the outstandingly superior effectiveness of the preferred additives as compared with the remainder of the additives of this invention.

To still further illustrate the thermal stability properties of the preferred jet fuels of this invention, additional tests were carried out. In these the base fuel was a commercially-available, straight-run kerosene jet fuel. In the above tests, this additive-free base fuel caused a pressure drop of 25 inches of mercury within the first 49 minutes of the test period. The merit rating of this base fuel was 92 and the preheater deposits which formed ranged from a haze to a brown coloration. The presence in the base fuel of only 0.007 percent by weight of 4-amino-2-methyl-6-tert-butyl phenol resulted in a filter test time virtually 300 percent as long as the additive-free base stock. Moreover, this extremely small quantity of a particularly preferred additive provided a merit rating of 254. Significantly, after completion of the test the particularly preferred fuel of this invention afforded an absolutely deposit-free preheater tube. In other words, on completion of the stringent test procedure, a very careful examination of the preheater tube showed it to be absolutely free from any detectable deposits or even haze.

It will be clearly apparent from the above that the present invention has now made possible the effective and efficient utilization of jet fuels even under the most drastic jet engine operating conditions.

Typical additives which can be used in the practice of this invention include such compounds as

4-amino-2,6-dimethyl phenol;

- 4-amino-2,6-diethyl phenol,
- 4-amino-2,6-diisopropyl phenol,
- 4-amino-2,6-di-sec-butyl phenol,
- 4-amino-2,6-di-(2-ethyl) phenol,
- 4-amino-2,6-di-(2-octyl) phenol,
- 4-amino-2,6-di-(3-dodecyl) phenol,
- 4-amino-2-methyl-6-(1,1,3,3-tetramethylbutyl) phenol,
- 4-amino-2-isopropyl-6-(1,1,2,2-tetramethyl) phenol,
- 4-amino-2,6-dicyclohexyl phenol,
- 4-amino-2,6-di-(1-phenylethyl) phenol,
- 4-(N-methylamino)-2-methyl-6-isopropyl phenol,
- 4-(N-butylamino)-2,6-diisopropyl phenol,
- 4-(N-isoctylamino)-2,6-di-(2-dodecyl) phenol,
- 4-(N-cyclohexylamino)-2,6-dicyclohexyl phenol,
- 4-(N-benzylamino)-2,6-diethyl phenol,
- 4-(N,N-diethylamino)-2-methyl-6-(2-heptyl) phenol,
- 4-(N,N-dibutylamino)-2-methyl-6-(2-decyl) phenol,
- 4-(N,N-dicyclohexylamino)-2,6-disopropyl phenol,
- 4-(N,N-dibenzylamino)-2-methyl-6-isopropyl phenol,
- 4-(N-octyl-N-benzylamino)-2,6-dimethyl phenol,

and the like.

Preferred additives of this invention are exemplified by such compounds as

- 4-amino-2-methyl-6-tert-amyl phenol,
- 4-amino-2-isopropyl-6-tert-amyl phenol,
- 4-amino-2-(2-dodecyl)-6-tert-amyl phenol,
- 4-(N-ethylamino)-2-ethyl-6-tert-butyl phenol,
- 4-(N-amylamino)-2,6-di-tert-amyl phenol,
- 4-(N-cyclohexylamino)-2-isopropyl-6-tert-butyl phenol,
- 4-(N-(4-methylbenzyl)amino)-2-methyl-6-tert-butyl phenol,
- 4-(N,N-diisopropylamino)-2,6-di-tert-butyl phenol,
- 4-(N,N-diethylamino)-2-methyl-6-tert-amyl phenol,
- 4-(N,N-dibenzylamino)-2-ethyl-6-tert-amyl phenol,
- 4-(N-methyl-N-cyclohexylamino)-2,6-di-tert-butyl phenol,

and the like.

Particularly preferred jet fuel thermal stabilizers of this invention are typified by such compounds as 4-amino-2-methyl-6-tert-butyl phenol, 4-amino-2-ethyl-6-tert-butyl phenol, 4-amino-2-isopropyl-6-tert-butyl phenol, 4-amino-2-propyl-6-tert-butyl phenol, 4-amino-2-nonyl-6-tert-butyl phenol, 4-amino-2-(2-dodecyl)-6-tert-butyl phenol, 4-amino-2,6-di-tert-butyl phenol, and the like.

The preparation of the vast majority of the jet fuel additives of this invention preferably involves the use of the aromatic-substitution process disclosed in our co-pending application, Serial No. 426,556, filed April 29, 1954, now Patent No. 2,831,898. According to one aspect of this process, phenol or phenols in which at least one ortho position is unsubstituted can be readily alkylated with olefins, cycloolefins, or aromatic substituted olefins so that one or two hydrocarbon substituents can be selectively introduced in the position or positions ortho to the hydroxyl group. Thus, by carrying out this process under the conditions described in our co-pending application, 2,6-dihydrocarbon-substituted phenols are readily prepared in high yield and in high purity even when starting with phenols having an unsubstituted para position. Typical of these are 2,6-di-tert-butyl phenol (from phenol and isobutylene), 2-methyl-6-tert-butyl phenol (from o-cresol and isobutylene), 2,6-di-isopropyl phenol (from phenol and propylene), 2-(2-dodecyl)-6-isopropyl phenol (by reacting phenol with a molar equivalent of propylene followed by reaction between o-isopropyl phenol and dodecane-1), 2-ethyl-6-cyclohexyl phenol (from 2-ethyl phenol and cyclohexene), 2,6-di-(1-phenylethyl) phenol (from phenol and styrene), 2-n-hexyl-6-(1,1,3,3-tetramethylbutyl) phenol (from 2-n-hexyl phenol and diisobutylene), etc. These 2,6-dihydrocarbon-substituted phenols which are either readily prepared by our aromatic-substitution process or prepared by other chemical means are intermediates for the preparation of the jet fuel thermal stabilizers of this invention.

The preparation of the jet fuel additives of this invention involves carrying out any of a number of chemical reactions using these 2,6-dihydrocarbon-substituted phenols. One such process is to selectively nitrate the 2,6-dihydrocarbon-substituted phenol to obtain the corresponding 4-nitro-2,6-dihydrocarbon-substituted phenol. This nitro compound is then reduced to form the unsubstituted 4-amino additives of this invention. On the other hand, the nitro compound can be subjected to reductive alkylation using an aldehyde or ketone containing up to about 8 carbon atoms, the structure of which governs the type of substituent or substituents which are thereby attached to the nitrogen atom. By using an aldehyde and appropriately adjusting the reaction conditions, one or two substituents are introduced onto the nitrogen atom. Thus, straight or branched primary alkyl groups result from the use of a straight or branched chain aliphatic aldehyde. Aralkyl groups are formed by using an aldehyde containing an aromatic group. When a ketone is used, one substituent is introduced onto the nitrogen atom and this substituent is either a secondary alkyl group (using an aliphatic ketone) or a cycloalkyl group (using a cycloaliphatic ketone).

In achieving selective para position nitration of the 2,6-dihydrocarbon-substituted phenol intermediates, it is particularly important to use highly specialized reaction conditions. In fact, it is imperative to use these critical reaction conditions when the ortho substituents on the phenol intermediates are easily removed such as by dealkylation. The reason for this is that these 2,6-dihydrocarbon-substituted phenols, for the most part, are readily dealkylated or totally destroyed under conventional nitration reaction conditions. For example, Hart and Cassis, J. Am. Chem. Soc., 73, 3179 (1951) have shown that when 2,6-di-tert-butyl phenol is nitrated with a mixture of nitric and acetic acids, dealkylation occurs with the resultant formation of 2-tert-butyl-4,6-dinitro phenol. It has also been found that in attempting to nitrate such phenols as 2,6-di-tert-butyl phenol with a nitration mixture composed of nitric and sulfuric acids, complete deterioration of the phenol is encountered as evidenced by the formation of large amounts of resins and tars.

This selective nitration process involves nitrating the 2,6-dihydrocarbon-substituted phenol with nitric acid in the presence of an inert hydrocarbon solvent, such as isooctane or benzene. In this process the best results are obtained when the di-ortho-substituted phenol dissolved in a hydrocarbon solvent is added to the nitric acid ranging in concentration from 30 to 70 percent, preferably from about 30 to 40 percent. The most satisfactory product is obtained with from 1.5 to 2.0 theories of nitric acid based on the amount of the 2,6-dialkyl phenol used. The reaction temperatures range from about 0 to about 40° C., the best results being obtained at a temperature range of 20 to 30° C. Yields in the order of about 80 percent of the nitro phenol of a purity in the range of about 95 to 97 percent have been achieved in this process.

Catalytic reduction of the resultant nitro phenol to form the 4-amino-2,6-dihydrocarbon-substituted phenol is readily carried out with a variety of reducing catalysts. However, it has been found that the most successful are nickel catalysts which contain a relatively high percentage of nickel oxide which apparently provides a highly active source of freshly reduced nickel. Concentrations as low as 2 percent by weight of such catalyst can be employed with excellent results. Hydrogen pressures in the range of 200 to 500 p.s.i. are satisfactory, the temperature ranging from about 20 to about 130° C. An alcohol solvent—methanol, ethanol, isopropanol, etc.—is generally employed.

Generally similar reaction conditions are employed in the reductive alkylation of the 4-nitro-2,6-dihydrocarbon-substituted phenols to form the nitrogen-substituted addi-

tives of this invention. In this instance a very useful catalyst is finely-ground platinum-on-silica gel. Good results are achieved by using 1 to 5 percent of the catalyst. The hydrogen pressures and reaction temperatures are essentially the same as in the case of the catalytic reductions discussed above. When the aldehyde or ketone has a relatively low molecular weight, it is desirable to use an excess which acts as a solvent.

Another way of preparing the above compounds which have one nitrogen substituent involves condensation of aldehydes or ketones with the unsubstituted 4-amino-2,6-dihydrocarbon-substituted phenols. This reaction results in the elimination of water which is conveniently removed from the reaction zone by use of a solvent which forms an azeotrope with water, such as benzene, toluene, xylene, etc. Formed are derivatives of the phenols which have a para-substituted nitrogen doubly bonded to the hydrocarbon group formed from the aldehyde or ketone used, i.e., a Schiff's base. These derivatives are reduced to the corresponding mono-substituted 4-amino-2,6-dihydrocarbon-substituted phenols by either catalytic or chemical means.

A generally applicable process of preparing the N-mono- and N,N-di-substituted additives of this invention is the reaction between the unsubstituted 4-amino-2,6-dihydrocarbon-substituted phenols and alkyl halides (primary, secondary, or tertiary), cycloalkyl halides or aralkyl halides. Hydrogen halide is given off in this reaction and it is thus desirable to use a hydrogen halide acceptor, such as pyridine, triethylamine, or the like. The use of about a mole of the organic halide per mole of the phenol favors the formation of the mono-substituted compounds, whereas an excess—i.e., 2 to 3 moles of the halide per mole of the phenol—results in di-substitution.

Another way of preparing the unsubstituted 4-amino additives of this invention involves coupling diazosulfanilic acid with the 2,6-dihydrocarbon-substituted phenol intermediate followed by reductive fission of the azo linkage to form the unsubstituted amino group. A number of common reagents are capable of bringing about this reductive fission. One convenient material is sodium hydrosulfite. According to this over-all method, the phenol is coupled with diazosulfanilic acid in a cold aqueous solution. After this reaction has been completed, sodium hydrosulfite is added and the temperature raised to 70 to 90° C. with the formation of the 4-amino additive which is separated by conventional means.

To still further illustrate the preparation of the compounds of this invention, reference is made to the following specific examples in which all parts and percentages are by weight, unless otherwise specified.

#### EXAMPLE 21

Preparation of 4-nitro-2,6-di-tert-butyl phenol.—In a reaction vessel equipped with stirring, condensing, temperature regulating and reagent introducing means was placed a solution of 103 parts of 2,6-di-tert-butyl phenol (prepared as described in our co-pending application, Serial No. 426,556, now Patent No. 2,831,898) in 350 parts of isooctane. Over a period of 11 minutes, 63 parts of 50 percent nitric acid was added at 20° C. The temperature was kept below 30° C. and after 2 minutes, a solid began to precipitate. The stirring was continued until a temperature drop was noted and then the solids were filtered off. This material was washed very thoroughly with water and dried to give 62.4 parts (50 percent yield) of crude 4-nitro-2,6-di-tert-butyl phenol, M.P. 145-153° C. This material crystallized from isooctane as white needles, M.P. 155.5-156° C.

Analysis.—Calculated for  $C_{14}H_{21}NO_3$ : 66.91% carbon; 8.42% hydrogen and 5.57% nitrogen. Found: 67.20% carbon; 8.36% hydrogen and 5.53% nitrogen. The molecular weight was found to be 257 with the theoretical being 251.3.

## 11

## EXAMPLE 22

*Preparation of 4-nitro-2-methyl-6-tert-butyl phenol.*—Into a reaction vessel were charged 60 parts of 70 percent nitric acid and 45 parts of water. To this was added with cooling and agitation 110 parts of 2-methyl-6-tert-butyl phenol dissolved in 50 parts of n-hexane. The temperature was maintained at 25-30° C. Additional quantities of hexane were added (50 parts total) in small portions as solids separated from the organic phase. The reaction mixture was filtered and washed with water, a dilute aqueous sodium bicarbonate solution and cold hexane to yield, after air drying, 71 parts (50 percent yield) of yellow solids melting at 139-142° C. This product was found to be 4-nitro-2-methyl-6-tert-butyl phenol.

## EXAMPLE 23

*Preparation of 4-nitro-2-decyl-6-tert-amyl phenol.*—Using the procedure as described in Example 21, a total of 76 parts of 2-decyl-6-tert-amyl phenol in 150 parts of benzene is treated with 32 parts of 50 percent nitric acid. The temperature is kept below 30° C. and the solids formed are filtered off, washed thoroughly and dried to give 4-nitro-2-decyl-6-tert-amyl phenol.

The methods of preparing the 4-nitro intermediates of the additives of this invention will now be apparent to those skilled in the art. Thus, these nitration procedures can be applied to such phenols as 2-methyl-6-cyclohexyl phenol; 2,6-di-(4-methylcyclohexyl) phenol; 2-propyl-6-benzyl phenol; 2,6-di(1-phenylethyl) phenol; and the like, to form the corresponding 4-nitro derivatives.

## EXAMPLE 24

*Preparation of 4-amino-2,6-di-tert-butyl phenol.*—To a rocking autoclave was charged the following mixture: 25.1 parts of 4-nitro-2,6-di-tert-butyl phenol, 3.0 parts of ground platinum-on-silica gel catalyst, and 105 parts of absolute ethanol. The autoclave was sealed, pressured to 200 p.s.i.g. with hydrogen and heated to 105° C. While maintaining the temperature at this level and operating at 300-500 p.s.i.g. of hydrogen, a total pressure drop of 780 p.s.i. was observed over a one-hour period. The autoclave was cooled, opened and the contents immediately filtered by suction to remove the catalyst. The solvent was removed from the red filtrate at reduced pressure. The crude 4-amino-2,6-di-tert-butyl phenol, which remained, weighed 20.5 parts (93 percent theory). Recrystallization from isoctane gave pink needles, M.P. 105-107° C.

*Analysis.*—Calculated for  $C_{14}H_{23}ON$ : 76.1% carbon; 10.5% hydrogen. Found: 76.1% carbon; 10.3% hydrogen. Infrared analyses and volumetric analyses for nitrogen confirmed the structure of this compound.

## EXAMPLE 25

*Preparation of 4-(N-sec-butylamino)-2,6-di-tert-butyl phenol.*—A mixture of 25.1 parts of 4-nitro-2,6-di-tert-butyl phenol, 3.0 parts of ground platinum-on-silica gel catalyst and 107 parts of methylethyl ketone was charged to a rocking autoclave. A pressure of 200 p.s.i.g. of hydrogen was applied and the reactants were heated to 105° C. After three hours of operation in the range of 300-500 p.s.i.g., a total pressure drop of 3520 p.s.i. was observed. The reaction was terminated, and the autoclave was cooled and discharged through a filter. The filtrate was vacuum distilled to give a considerable amount of 2-butanol followed by 22.7 parts (82 percent theory) of a viscous, red oil, B.P. 136-137° C. at a pressure of less than one millimeter.

*Analysis.*—Calculated for  $C_{18}H_{31}ON$ : 78.1% carbon; 11.3% hydrogen. Found: 77.9% carbon; 11.1% hydrogen. Infrared analyses and basic nitrogen titration confirmed the structure of the product.

## EXAMPLE 26

*Preparation of 4-(N,N-dibenzylamino)-2,6-di-tert-butyl phenol.*—A mixture of 25.1 parts of 4-nitro-2,6-di-

5

10

tert-butyl phenol, 30 parts of benzaldehyde and 3.0 parts of platinum-on-silica gel catalyst is placed in 200 parts of methanol and charged to a rocking autoclave. At a hydrogen pressure of 400 to 500 p.s.i.g., the reactants are reduced over a period of three hours. The reaction is carried out between 100 and 140° C. At the end of the reaction, the autoclave is cooled, discharged through a filter and the filtrate evaporated using an aspirator. The residue is taken up in ether, washed with aqueous sodium bicarbonate and the organic phase evaporated to give 4-(N,N-dibenzylamino)-2,6-di-tert-butyl phenol.

## EXAMPLE 27

*Preparation of 4-(N-cyclohexylamino)-2-ethyl-6-tert-butyl phenol.*—A mixture of 22.3 parts of 4-nitro-2-ethyl-6-tert-butyl phenol in 50 parts of cyclohexanone and 50 parts of ethanol is hydrogenated at 150 to 180° C. using a copper chromite catalyst. Hydrogen absorption is complete after five hours of operation in the range of 400 to 500 p.s.i.g. The autoclave is cooled and the contents filtered to remove the catalyst. Vacuum distillation of the filtrate gives the desired 4-(N-cyclohexylamino)-2-ethyl-6-tert-butyl phenol.

15

20

25

30

35

40

45

50

55

60

65

70

75

## 12

## EXAMPLE 28

*Preparation of 4-(N-isobutylamino)-2-methyl-6-tert-amyl phenol.*—78 parts of isobutyraldehyde is rapidly added with stirring to 150 parts of 4-amino-2-methyl-6-tert-amyl phenol suspended in 500 parts by volume of 50 percent methanol at ambient temperatures. The temperature of the reaction mixture increases and upon cooling a precipitate appears. 50 parts of the resulting Schiff's base together with 20 parts of a nickel catalyst and 100 parts of toluene are shaken at 125 to 135° C. under 500 p.s.i.g. hydrogen pressure until no more hydrogen is absorbed. The charge is then cooled, filtered and the filtrate distilled under reduced pressure. A viscous, red oil, 4-(N-isobutylamino)-2-methyl-6-tert-amyl phenol, is obtained in this manner.

The amount of the additive used in the jet fuels of the invention can range from about 0.001 to about 0.5 percent by weight. Concentrations of from about 0.01 to about 0.1 percent are preferred, especially when using the preferred additives of this invention. Variations from these concentration ranges are permissible. For example, in jet fuel initially possessing a fair degree of thermal stability very small amounts of the additives (0.001 to about 0.06 percent) are sufficient to greatly improve the thermal stability characteristics of such fuels. On the other hand, where the jet fuel initially has a very poor thermal stability, larger amounts (about 0.1 to about 0.5 percent by weight or more) can be effectively used.

In preparing the improved jet fuels of this invention, the use of solvents for the additives is helpful. While solubility of these additives in jet fuels is very high, especially in the case of the preferred and particularly preferred additives, blending procedures are simplified by pre-dissolving these thermal stabilizers in a suitable solvent. The resulting formulations can then be conveniently and readily blended with the jet fuel. One good way of accomplishing this is to pre-dissolve an additive of this invention in high concentration in a small portion of the jet fuel to be thermally stabilized. This concentrated solution (for example, 10 percent by weight of the additive) is then dissolved with the remainder of the jet fuel to provide the concentration desired. Other particularly suitable solvents for this purpose include benzene, toluene, xylene, acetone, methylethyl ketone, methanol, ethanol, isopropanol, methyl isobutyl carbinol, and the like. In general ketones and alcohols containing up to about 6 carbon atoms and liquid aromatic hydrocarbons containing 6 to 18 carbon atoms are excellent solvents. Other materials that can be used in the jet fuels of this invention are anti-rust

additives, dispersants, and, in general, additives which do not adversely affect the high-temperature stability of the fuels.

We claim:

1. Jet fuel distillate having an endpoint of at least about 480° F. containing from about 0.001 to about 0.5 percent by weight of 4-amino-2,6-dihydrocarbon-substituted phenol having the general formula



wherein R<sub>1</sub> and R<sub>2</sub> are selected from the group consisting of alkyl, cycloalkyl, and aralkyl groups containing up to about 12 carbon atoms each, and R<sub>3</sub> and R<sub>4</sub> are selected from the group consisting of hydrogen, alkyl, cycloalkyl and aralkyl groups containing up to about 8 carbon atoms.

2. A process for cooling the lubricating oil in a jet engine comprising using as a coolant for heat transfer with the lubricating oil a thermally stabilized jet fuel consisting essentially of a distilled hydrocarbon fuel having an endpoint of at least about 480° F. and containing from about 0.001 to about 0.5 percent by weight of a 4-amino-2,6-di-hydrocarbon-substituted phenol having the formula



wherein R<sub>1</sub> and R<sub>2</sub> are selected from the group consisting of alkyl, cycloalkyl, and aralkyl groups containing up to about 12 carbon atoms each, and R<sub>3</sub> and R<sub>4</sub> are selected from the group consisting of hydrogen, alkyl, cycloalkyl and aralkyl groups containing up to about 8 carbon atoms.

3. The composition of claim 1 in which said 4-amino-2,6-dihydrocarbon-substituted phenol is a 2,6-dialkylphenol wherein the alkyl groups are tertiary groups containing 4 to 5 carbon atoms each.

4. The composition of claim 1 wherein said 4-amino-2,6-dihydrocarbon-substituted phenol is a 2,6-dialkylphenol wherein one of the alkyl groups contains no more than about 12 carbon atoms and the other alkyl group is a tertiary butyl group.

5. The composition of claim 3 in which said 4-amino-2,6-dialkylphenol is a 4-amino-2,6-di-tert-butylphenol.

6. The process of claim 2 in which said 4-amino-2,6-di-hydrocarbon-substituted phenol is a 4-amino-2,6-di-alkylphenol in which the alkyl groups are tertiary groups and contain 4 to 5 carbon atoms each.

7. The process of claim 6 wherein said 4-amino-2,6-di-alkylphenol is a 4-amino-2,6-di-tert-butylphenol.

25 References Cited in the file of this patent

UNITED STATES PATENTS

|           |                  |       |               |
|-----------|------------------|-------|---------------|
| 2,074,467 | Gutzeit          | ----- | Mar. 23, 1937 |
| 2,250,501 | Rosenwald et al. | ----- | July 29, 1941 |
| 2,571,091 | Wasserman et al. | ----- | Oct. 16, 1951 |
| 2,712,497 | Fox et al.       | ----- | July 5, 1955  |